

## UNITED STATES PATENT OFFICE

GEORGE L. BIDWELL, OF RIEGELSVILLE, PENNSYLVANIA, ASSIGNOR TO RIEGEL PAPER CORPORATION, OF RIEGELSVILLE, NEW JERSEY, A CORPORATION OF NEW JERSEY

## PAPER

No Drawing.

Application filed May 10, 1932. Serial No. 610,505.

This invention relates to paper, and particularly to paper, such as glassine, imitation parchment and the like, made from stock of highly gelatinized fibers; and the object thereof is to improve the transparency, pliability, and other desirable characteristics in paper of this type.

In the manufacture of these papers in a standard Fourdrinier paper-making machine, 10 the paper stock is caused to flow on the Fourdrinier wire where the web is formed and a portion of the water is extracted therefrom first by capillary attraction as the web passes over tube rolls and then by suction as it 15 passes over the usual flat suction-boxes and the final suction couch roll. From the Fourdrinier wire the web is conducted, upon one or more, usually three, endless felt carriers, first between lower suction and top press 20 rolls and then between one or more pairs of standard press rolls by which more water is mechanically pressed from the web. On leaving the last of these rolls the web passes over and around a preliminary pair of 25 smoothing rolls and then over and around an extended battery of steam drying cylinders which serve to evaporate out most of the moisture contained therein. If the paper is to be sized a size press is inserted at the end 30 of the battery of drying cylinders and a few more drying cylinders are added to remove some or all of the moisture taken up by the paper web from the size press, the number 35 of the extra cylinders used depending upon the grade of paper to be made. The paper web or sheet thus dried is then passed through a pair of calendar rolls and wound up into rolls upon reels; and as each roll of 40 paper is completed the reel is removed and set in bearings on a frame and the paper is unreeled and run through a slitting and winding machine. Imitation parchment paper is a finished product at this stage, but, 45 in the case of glassine, the paper requires further treatment which consists in dampening it, by passing it through a mechanical dampener, then running it through super-calendars to give it a high finish and partial 50 transparency, and is usually waxed by run-

ring it through a waxing machine to render it waterproof and still more transparent.

I have found that I can enhance the physical properties or characteristics of the paper by incorporating therein, during its manufacture, small percentages of a mild alkali like sodium meta-silicate, cerelose or its equivalent in grape sugar, glucose, or dextrose, or a combination of two or more of these materials, and a plasticizer like glycerin, glycol, magnesium chloride, or zinc chloride as by running the sheet when partially dried but while still holding a considerable percentage of moisture through a size-press containing an aqueous solution of these materials. The cerelose or its equivalent improves the transparency, glossy surface, silver whiteness, flatness, and grease-proof qualities of the paper, while the mild alkali adds to the sheen and the plasticizer serves, when thus applied, to give the paper pliability and more or less stretch and in the case of the chloride of magnesium or zinc also adds to the weight of the sheet, and the degree of these characteristics in the finished paper can be controlled by varying the percentages of the ingredients and by diluting the solution more or less with water.

Attempts have been made to incorporate these various materials in the paper web both before it reaches and after it leaves the drying cylinders. Such attempts, however, have proven either unsatisfactory or uncommercial. For example, if the paper web is passed through the solution when nearly dry it will take up very large quantities thereof and the excess will have to be dried out again. Decidedly the best results are obtained by dividing the battery of drying cylinders into two sections and installing between them a size-press through which the sheet is run and subjected to a bath of the impregnating solution, preferably bringing the paper to the first section of dryers with a moisture content of approximately 82 per cent. and so dividing the battery that the cylinders in the first section will remove about 14 to 22 of such 82 per cent. moisture content, leaving the sheet with about 60 to 68 percent. of moisture at the time it is treated with the solution in the size-press.

The sheet will subsequently lose all except approximately 5 per cent. of its moisture in passing through the second section of the drying battery, and this moisture content will 5 be increased to approximately 7 per cent. by subjecting its surfaces to the action of a pair of cooling rolls before the sheet is reeled. The ordinary size press and extra drying cylinders, if used, should be inserted between the 10 second section of the drying battery and the cooling rolls.

For the impregnating bath I now prefer, and recommend, cerelose as the material for enhancing what may be termed the visual 15 characteristics of the paper, and glycerin as the plasticizer to give it pliability and stretch, and highly satisfactory results have been obtained from using in the size-press a solution composed, approximately, either of 20 per 20 cent. cerelose, 4 per cent. sodium meta-silicate, 20 per cent. glycerin, and 56 per cent. water or of 50 per cent. cerelose, 4 per cent. sodium meta-silicate, 20 per cent. glycerin, and 26 per cent. water. A still more plastic sheet is obtained by the use of a solution with 30 per 25 cent. cerelose, 4 per cent. sodium meta-silicate, 10 per cent. magnesium or zinc chloride, 20 per cent. glycerin, and 36 per cent. water, while a very handsome sheet can be made 30 with as simple a solution as 20 per cent. cerelose, 20 per cent. glycerin, and 60 per cent. water. However, if very good plastic qualities are required, the heavier solutions are more 35 desirable. The sodium meta-silicate adds sheen to the sheet and hence it is desirable, although not essential, to use it in the impregnating bath in the size-press as well as in the water with which glassine paper is later dampened as will now be explained.

40 I have also found that the transparency and glossiness or sheen of surface of glassine paper can be further enhanced by thoroughly and evenly dampening the sheet, preparatory to passing it through the supercalenders, with alkali treated water—for example, water having dissolved therein approximately 2 to 5 per cent. of sodium meta-silicate or its equivalent, preferably dampening one 45 side of the sheet both by passing it through 50 a mechanical dampener and over an air-operated atomizer, then brushing the water thoroughly over and intimately in contact with the fibers of the sheet, and then rolling the sheet into a tight roll. The paper when 55 so treated takes on a very high gloss and becomes exceedingly transparent on passing through the supercalenders, and it is further improved in these respects when waxed and, especially, when run through a waxing 60 machine using a wax of a very high temperature.

It will, of course, be understood that the invention can be modified in its various details, within the scope of the appended 65 claims, without departing from the spirit

or sacrificing the substantial advantages thereof.

What I claim as new, and desire to secure by Letters Patent, is—

1. Paper of the type described treated 70 with an aqueous solution of cerelose.
2. Paper of the type described treated, with an aqueous solution of cerelose and glycerin.
3. Paper of the type described treated 75 with an aqueous solution of cerelose, sodium meta-silicate, and a plasticizer.
4. Paper of the type described having incorporated therein before the drying of the web has been completed a material like 80 cerelose adapted to enhance its transparency.
5. Paper of the type described having incorporated therein before the drying of the web has been completed a material like 85 cerelose adapted to enhance its transparency and a plasticizer like glycerin.
6. Paper of the type described having incorporated therein before the drying of the web has been completed a material like 90 cerelose adapted to enhance its transparency, a material like sodium meta-silicate adapted to enhance its sheen, and a plasticizer.
7. Paper of the type described containing the materials incorporated therein by the treatment thereof before the drying of the 95 sheet has been completed with a solution containing approximately 20 to 50 per cent. cerelose, 20 to 35 per cent. of a plasticizer, and 15 to 60 per cent. of water.
8. Paper of the type described containing the materials incorporated therein by the treatment thereof before the drying of the sheet has been completed with a solution containing approximately 20 to 40 per cent. of 100 cerelose, 2 to 5 per cent. of sodium meta-silicate, 15 to 35 per cent. of a plasticizer, and 20 to 63 per cent. of water.
9. Glassine paper having incorporated 105 therein a material like cerelose adapted to enhance its transparency and a plasticizer like glycerin, and dampened preparatory to being supercalendered with water containing a small percentage of an alkali like sodium meta-silicate.
10. Glassine paper having incorporated 110 therein before the drying of its web has been completed a material like cerelose adapted to enhance its transparency and a plasticizer, dampened preparatory to being supercalendered with water containing a small percentage of an alkali like sodium meta-silicate, and waxed with a high temperature wax.
11. Glassine paper having incorporated 115 therein before the drying of its web has been completed a material like cerelose adapted to enhance its transparency, an alkali like sodium meta-silicate adapted to enhance its sheen, and a plasticizer, and dampened 120 preparatory to being super-calendered.
12. Glassine paper having incorporated 125 therein before the drying of its web has been completed a material like cerelose adapted to enhance its transparency, an alkali like sodium meta-silicate adapted to enhance its sheen, and a plasticizer, and dampened 130 preparatory to being super-calendered.

12. Glassine paper having incorporated therein before the drying of its web has been completed a material like cerelose adapted to enhance its transparency and a plasticizer, 5 and waxed with a high temperature wax.

13. Glassine paper having incorporated therein from an aqueous solution before the drying of its web has been completed with a material like cerelose, an alkali like sodium 10 meta-silicate, and a plasticizer, and waxed with a high temperature wax.

14. Glassine paper having incorporated therein from an aqueous solution before the drying of its web has been completed with 15 materials like cerelose, sodium meta-silicate, and a plasticizer, dampened preparatory to being supercalendered with water containing an alkali like sodium meta-silicate, and waxed with a high temperature wax.

20 GEORGE L. BIDWELL.

26

30

35

40

45

50

55

60

65